

1

3,411,996

## PROCESS FOR BRIGHTENING ZINC AND CADMIUM ELECTROPLATE USING AN INNER SALT OF A QUATERNIZED PYRIDINE CARBOXYLIC ACID AND COMPOSITIONS CONTAINING THE SAME

John D. Rushmere, Wilmington, Del., assignor to E. I. du Pont de Nemours and Company, Wilmington, Del., a corporation of Delaware

No Drawing. Continuation-in-part of application Ser. No. 511,245, Dec. 2, 1965. This application Sept. 20, 1967, Ser. No. 669,309

16 Claims. (Cl. 204—50)

## ABSTRACT OF THE DISCLOSURE

It has been found that the addition of an inner salt of a quaternized pyridine carboxylic acid to aqueous alkaline electroplating baths containing zinc and cadmium ions provides smooth, bright deposits of these metals. High plating efficiency with low consumption of the inner salt of the quaternized pyridine compound is obtained using it alone or in combination with other bath additives.

## CROSS REFERENCES TO RELATED APPLICATIONS

This application is a continuation-in-part of application Ser. No. 511,245 filed Dec. 2, 1965, now abandoned.

## SUMMARY OF INVENTION

According to the present invention there is provided an aqueous, alkaline electroplating bath containing metal ions selected from the group consisting of zinc and cadmium having the improvement comprising an inner salt of a quaternized pyridine carboxylic acid having the formula



wherein R is hydrogen or



dissolved therein in an amount to yield a metal deposit of improved brightness.

The invention also comprises the process for electroplating zinc and cadmium from an aqueous, alkaline electroplating bath which comprises adding to the bath from about 0.1 to about 10 grams/liter of an inner salt of a quaternized pyridine carboxylic acid of the above formula.

The invention is also an aqueous addition agent for an electroplating bath containing zinc or cadmium ions comprising from about 1:100 to 100:1 parts by weight of an inner salt of a quaternized pyridine carboxylic acid of the above formula and a bath soluble organic polymer.

## DETAILED DESCRIPTION OF INVENTION

The inner salt of a quaternized pyridine carboxylic acid must be soluble in the bath, i.e., having a solubility of at least about 0.01 gram/liter at a temperature of about 25° C. The compounds may be obtained from commercial

2

sources or may be prepared by quaternizing a pyridine carboxylic acid. The inner salt of a quaternized pyridine compound is readily prepared from acids of pyridine, many of which are commercially available, and quaternizing agents which are usually benzyl halides. The inner salts may also exist as dimers or higher condensed forms.

The inner salt of a quaternized pyridine carboxylic acid used in the present invention has the formula



wherein R is hydrogen or



Preferred compounds are 1-benzyl pyridinium 3-carboxylate and p-xylylene bis(pyridinium 3-carboxylate).

The quaternized pyridine inner salts are preferably used in combination with organic polymers which are also soluble in the bath. The presence of the polymer is particularly desirable when the bath is used at temperatures above room temperature. The quaternized pyridine inner salt may generally be used alone at a temperature from about 20° C. to 30° C.; however, at the higher temperatures, i.e., 30° C. to 50° C., it is usually desirable to use both a quaternized pyridine inner salt and an organic polymer.

Examples of suitable polymers include synthetic polymers such as polyvinyl alcohol and polyethylene amine, and natural polymers such as gelatin, glue, peptone, gum tragacanth, gum arabic, gum ghatti, gum guaiac, and agar-agar as well as protein substances such as egg albumin and milk protein hydrolysate. The polyvinyl alcohol may be modified, e.g., a partial ether formed by condensation with ethylene oxide or glycidol. The polyvinyl alcohols prepared by hydrolysis of polyvinyl acetate are a preferred type of organic polymer. Those having average molecular weights from about 5,000 to 20,000 which are either fully hydrolyzed or partially hydrolyzed (87%—89%) provide particularly stable plating baths.

The brightening compositions of this invention are preferably used in the form of aqueous addition agents for the zinc and cadmium plating baths. Additives for the plating baths may be prepared containing from about 1:100 to 100:1 parts by weight of the quaternized pyridine inner salt and organic polymer. The addition agent preferably consists of an aqueous solution containing from about 5 to 35% by weight of solids and is added directly to the bath. Preferably, the additive will contain from about 3:1 to 9:1 parts by weight of quaternized pyridine inner salt to polymer.

In preparing the plating baths, zinc and cadmium ions are made available in the usual manner by adding oxides, hydroxides and cyanides of these metals to the plating bath. The bath should be alkaline in nature since the quaternized pyridine inner salts tend to be ineffective as brightening agents under acid conditions. In a preferred electroplating bath containing zinc or cadmium, from about 0.1 to 10 grams/liter of a quaternized pyridine inner salt will be present from about 0.01 to 10 grams/liter of the organic polymer.

The invention will be further illustrated by the following examples in which parts and percentages are by weight unless otherwise specified. In the examples both barrel and still plating operations were carried out.

## Example I

In a series of experiments, an aqueous plating bath having the following composition was prepared:

|                  | Grams/liter | 10 |
|------------------|-------------|----|
| Sodium cyanide   | 40          |    |
| Sodium hydroxide | 90          |    |
| Zinc cyanide     | 60          |    |
| Sodium carbonate | 80          |    |
| Sodium sulfide   | 1           |    |

1-benzyl pyridinium 3-carboxylate was prepared by quaternizing 1 mole of nicotinic acid (123 grams) with 1 mole of benzyl chloride (126 grams) in 400 grams of water. Sufficient sodium hydroxide was added to the reaction mixture to give a pH of 6.0 to 6.5. The mixture was then refluxed for three hours, cooled, and diluted to give a 10% by weight solution which was added to the cyanide plating bath.

*Test 1: Demonstrating wide brightness range.*—A steel Hull cell panel was plated at 2 amp. for 5 minutes in a bath containing 0.8 gram/liter of 1-benzyl pyridinium 3-carboxylate. After washing and a dip in 0.5 weight percent nitric acid to remove stains, an extremely bright plate was obtained over the current density range 4–150 amp./sq. ft. In a control experiment conducted in the absence of any additive, a uniformly dull plate over the entire face of the panel was obtained (1–150 amp./sq. ft.).

*Test 2: Demonstrating utility in practical still plating.*—A steel crank hole cover was plated at 2 amp. for 15 minutes in a cyanide plating bath containing 0.8 gram/liter of 1-benzyl pyridinium 3-carboxylate. After washing and a dip in 0.5 weight per cent nitric acid, an extremely bright shiny plate was obtained on all surfaces, even those of low current density.

*Test 3.*—Test 2 was repeated except that a series of crank hole covers were plated successively in the bath to which was added a partially hydrolyzed (87–89%) polyvinyl alcohol having a molecular weight of about 16,800 with the amount of polyvinyl alcohol being increased after each plating operation. The following observations were made on the plated products, demonstrating that even very small amounts of polyvinyl alcohol improve the quality of the electroplate over that obtained by either compound alone.

TABLE 1

|          | 1-benzyl<br>pyridinium<br>3-carboxylate<br>added, g./l. | Polyvinyl<br>alcohol<br>added, g./l. | Product quality                                                                                                   |
|----------|---------------------------------------------------------|--------------------------------------|-------------------------------------------------------------------------------------------------------------------|
| (a)----- | 0.8                                                     | 0                                    | Very desirable product. Bright on all surfaces.                                                                   |
| (b)----- | 0.8                                                     | 0.004                                | Brightness about the same as (a). Increase in shininess of plate.                                                 |
| (c)----- | 0.8                                                     | 0.04                                 | Product about the same as (b).                                                                                    |
| (d)----- | 0.8                                                     | 0.08                                 | Plate very bright and shiny. Improved over (b).                                                                   |
| (e)----- | 0.8                                                     | 0.13                                 | Plate has extremely bright and liquid appearance even in low current density areas. Over-all mirror-like quality. |
| (f)----- | 0                                                       | 0.13                                 | Dull on all surfaces.                                                                                             |

*Test 4: Demonstrating utility in practical barrel plating.*—One hundred grams steel screws were barrel plated at 3 amp. for 30 minutes in a zinc cyanide plating bath containing 0.8 gram/liter of 1-benzyl pyridinium 3-carboxylate. The screws produced were very shiny and showed little staining. They were not significantly improved in quality by a dip in 0.5 weight percent nitric acid.

## Example II

Example I was repeated except that 115 grams/liter of sodium cyanide were used in the bath and 30 grams/liter of cadmium oxide were substituted for the zinc cyanide.

*Test 5: Demonstrating brightness range.*—A steel Hull cell panel was plated at 1 amp. for 5 minutes in a cadmium cyanide plating bath containing 0.8 gram/liter of 1-benzyl pyridinium 3-carboxylate. After washing and a short dip in 0.5 weight percent nitric acid, a smooth bright plate was obtained over the range 10–60 amp./sq. ft.

A control panel plated under similar conditions but in the absence of the quaternized pyridinium inner salt had a dull white plate across the entire face of the panel.

*Test 6: Demonstrating utility in practical still plating.*—A steel Hull cell panel bent in the form of a rectangular Z shape was plated at 2 amp. for 15 minutes in a cyanide bath containing 0.5 gram/liter of 1-benzyl pyridinium 3-carboxylate. After bright dipping in a dilute  $H_2O_2$ — $H_2SO_4$  bright dip, the work showed a nice bright shiny plate extending all the way into the recesses of the Z which demonstrates the excellent throwing power of the plating bath.

By comparison, a control piece plated in the absence of the quaternized pyridinium inner salt showed a semi-bright matte plate.

## Example VI

In a series of experiments, an aqueous plating bath having the following composition was prepared:

|                  | Grams/liter |
|------------------|-------------|
| Sodium cyanide   | 40          |
| Sodium hydroxide | 90          |
| Zinc cyanide     | 60          |
| Sodium carbonate | 80          |

A series of inner salts quaternized pyridinium compounds were prepared by refluxing 0.1 mole of a pyridine carboxylic acid and an equimolar quantity of a quaternizing agent in 100 cc. of water. The reaction was judged as having taken place by the disappearance of the oily appearance of the quaternizing agent or change in color of the reflux. The mixture was cooled and then diluted to give a 10 weight percent solution of the resulting inner salt of a quaternized pyridinium compound. In the series of tests reported in Table 2 which follows, the quaternized pyridinium compound was added to the plating bath in an amount of about 0.8 gram/liter. All of the quaternized pyridinium compounds were found to be effective brightening agents.

50

TABLE 2

| Test No. | Pyridine Compound                   | Quaternizing Agent              |
|----------|-------------------------------------|---------------------------------|
| 7-----   | Pyridine 4-carboxylic acid          | Benzyl chloride.                |
| 8-----   | Pyridine 3,5-dicarboxylic acid      | Do.                             |
| 9-----   | Pyridine 3-carboxylic acid (2 mols) | <i>a,a'</i> -Dichloro p-xylene. |

What is claimed is:

1. In an aqueous alkaline electroplating bath containing metal ions selected from the group consisting of zinc and cadmium, the improvement which comprises an inner salt of a quaternized pyridine carboxylic acid having the formula

65



wherein R is hydrogen or



dissolved therein in an amount to yield a metal deposit of improved brightness.

2. The electroplating bath of claim 1 wherein the inner salt of a quaternized pyridine carboxylic acid is 1-benzyl pyridinium 3-carboxylate.

3. The electroplating bath of claim 1 wherein the inner salt of a quaternized pyridine carboxylic acid is p-xylylene bis(pyridinium 3-carboxylate).

4. The electroplating bath of claim 1 wherein the bath is a cyanide bath.

5. In the process for electrodepositing a metal from an aqueous alkaline electroplating bath containing metal ions selected from the group consisting of zinc and cadmium, the improvement which comprises having present in said bath from about 0.1 to about 10 grams/liter of an inner salt of a quaternized pyridine carboxylic acid having the formula



wherein R is hydrogen or



6. The process of claim 5 wherein the inner salt of a quaternized pyridine carboxylic acid is 1-benzyl pyridinium 3-carboxylate.

7. The process of claim 5 wherein the inner salt of a quaternized pyridinium carboxylic acid is p-xylylene bis(pyridinium 3-carboxylate).

8. The process of claim 5 wherein a bath soluble organic polymer is present in the bath in an amount from about 0.01 to about 10 grams/liter.

9. The process of claim 8 wherein the bath soluble organic polymer is a polyvinyl alcohol having a molecular weight between about 5,000 and 20,000.

10. The process of claim 5 wherein the electroplating bath is a cyanide bath.

11. An aqueous addition agent for an electroplating bath containing metal ions selected from the group consisting of zinc and cadmium consisting essentially of from

about 1:100 to 100:1 parts by weight of an inner salt of a quaternized pyridine carboxylic acid having the formula



wherein R is hydrogen or



and a bath soluble organic polymer.

12. The composition of claim 11 wherein said addition agent contains from about 5 to 35% by weight of solids.

13. The composition of claim 11 wherein the inner salt of a quaternized pyridine carboxylic acid is 1-benzyl pyridinium 3-carboxylate and the bath soluble organic polymer is a polyvinyl alcohol having a molecular weight between about 5,000 and 20,000.

14. The composition of claim 13 wherein the composition contains from about 3:1 to about 9:1 parts by weight of said 1-benzyl pyridinium 3-carboxylate to said polyvinyl alcohol.

15. The composition of claim 11 wherein the inner salt of a quaternized pyridine carboxylic acid is p-xylylene bis(pyridinium 3-carboxylate) and the organic polymer is a polyvinyl alcohol having a molecular weight between about 5,000 and 20,000.

16. The composition of claim 15 wherein the composition contains from about 3:1 to about 9:1 parts by weight of said p-xylylene bis(pyridinium 3-carboxylate) to said polyvinyl alcohol.

#### References Cited

##### UNITED STATES PATENTS

|           |        |                |       |           |
|-----------|--------|----------------|-------|-----------|
| 1,536,859 | 5/1925 | Humphries      | ----- | 204—50    |
| 2,080,520 | 5/1937 | Westbrook      | ----- | 204—55    |
| 2,171,842 | 9/1939 | Barrett et al. | ----- | 204—50 XR |
| 2,803,593 | 8/1957 | High et al.    | ----- | 204—50    |
| 3,317,412 | 5/1967 | Dahlmann       | ----- | 204—55    |
| 3,318,787 | 5/1967 | Rindt et al.   | ----- | 204—55    |

55 HOWARD S. WILLIAMS, *Primary Examiner.*

G. KAPLAN, *Assistant Examiner.*